

## UNITED STATES PATENT OFFICE

2,577,626

## PREVENTING CORROSION OF METALS

Cecil Phillips, Jr., Baytown, Tex., assignor, by  
mesne assignments, to Standard Oil Develop-  
ment Company, Elizabeth, N. J., a corporation  
of Delaware

No Drawing. Application June 20, 1947,  
Serial No. 756,112

5 Claims. (Cl. 23—193)

1

This invention is directed to a method for sup-  
pressing the corrosion of copper-containing  
alloys in the presence of ammonia. Specifically,  
it is directed to the prevention of corrosion of  
copper alloys in aqueous solutions containing  
ammonia.

In many operations it is often desirable to use  
various types of equipment (tanks, heat ex-  
changer and condenser tubes, valves, lines, etc.)  
constructed of or containing copper alloys for  
handling solutions or gases containing ammonia.  
Such equipment usually suffers from severe cor-  
rosion of the copper alloys due to the chemical  
dissolution of the copper by the ammonia. The  
rapid destruction of the copper alloys in con-  
tact with solutions or vapors containing ammonia  
is believed to be due to the formation of highly  
soluble copper-ammonium complex ions. The  
presence of oxygen is necessary for the forma-  
tion of the soluble copper-ammonium ions.

As a result of the corrosive action of ammoni-  
acal solutions on copper, the employers of am-  
monia, such as the petroleum refiner, must ex-  
ercise extreme care in selection of suitable alloys  
for his processing equipment. Thus, where am-  
monia is to be used, copper alloys are avoided.  
However, as mentioned before, various services  
require the use of copper alloys on account of  
other corrosive fluids being encountered. Thus  
the corrosive action of carbon dioxide in steam  
makes nearly mandatory the employment of  
copper alloys such as an alloy of copper, zinc,  
and tin in heat exchange equipment using cor-  
rosive steam as the heat transfer medium. Thus,  
when ammonia is employed in this type of equip-  
ment, rapid attack of the copper alloy may be  
suffered even though the ammonia may prevent  
attack of ferrous metals by other components  
travelling through the equipment. Ammoniacal  
solutions are also widely used in solvent extrac-  
tion of hydrocarbons. Here, again the petroleum  
refiner must guard against allowing the solutions  
to contact copper-bearing surfaces. The afore-  
mentioned corrosion reaction generally occurs at  
atmospheric temperature and pressure. It is  
believed that higher temperatures and pressures  
may accelerate this reaction.

It is, therefore, the main object of the present  
invention to provide a process whereby the  
deterioration of copper alloys in the presence of  
ammonia is substantially eliminated.

Another object of the invention is to provide  
a method whereby copper alloys may be em-  
ployed in services where they are exposed to  
ammoniacal solutions.

The objects of the present invention are  
achieved by maintaining in corrosive ammoniacal  
solutions in contact with copper and its alloys  
a corrosion inhibiting amount of a salt of a  
petroleum sulfonic acid.

Briefly, the present invention involves the

2

addition to corrosive ammoniacal solutions in  
contact with copper bearing metals of a quantity  
of a salt of petroleum sulfonic acid, such as an  
alkali metal salt of petroleum sulfonic acid, in the  
range between 0.001% to 5% by weight, based  
on the ammoniacal solution.

The salts of petroleum sulfonic acid which are  
suitable for use in the practice of the present  
invention are the alkali metal salts of petroleum  
sulfonic acids, such as the lithium, sodium, or  
potassium salts. The ammonium salts of petro-  
leum sulfonic acids are also eminently suitable  
in the practice of the present invention.

The petroleum sulfonic acids which are em-  
ployed to produce the salts used in the present  
invention may be obtained in a manner well  
known to the art. The production of mahogany  
sulfonic acids has been disclosed widely in patent  
literature. However, a conventional method for  
preparing these acids involves the treatment with  
concentrated sulfuric acid of a feed stock com-  
prising a substantial portion of unsaturated cyclic  
hydrocarbons. Exemplary of the type of feed  
stocks which may be used are the solvent extracts  
resulting from solvent extraction of a distillate  
boiling in the lubricating oil boiling range, such  
as, for example, a phenol extract. The extract  
layer, upon treatment with strong sulfuric acid  
results in the formation of a layer comprising  
oil and oil soluble sulfonic acids or mahogany  
acids, and a second layer comprising sludge par-  
ticles and water-soluble sulfonic acids. These  
two layers are then separated under the influ-  
ence of gravity and the oil layer, including  
mahogany acids, is treated with successive por-  
tions of water to obtain the predominately oil  
soluble sulfonic acids. These oil soluble sulfonic  
acids may be freed of water and then converted  
into the corresponding salts by addition of sodium  
hydroxide or ammonium hydroxide if desired.  
As a specific example, a distillate obtained from  
a naphthenic crude oil may be solvent extracted  
with a solvent having the characteristics of fur-  
fural or phenol and the extract brought in con-  
tact with sulfuric acid of approximately 98%  
concentration. Upon contacting the concen-  
trated sulfuric acid with the petroleum extract,  
sulfonic acids are formed. The mahogany acids  
remain in the oil phase which separates from the  
acid phase.

In applying the concentrated sulfuric acid, it  
is customary to divide the total amount em-  
ployed into a number of portions and treat the  
petroleum extract separately with each portion  
and the mahogany acids allowed to remain in  
the extract phase or separated, if desired, be-  
tween each treat with sulfuric acid. Preferably  
the oil soluble sulfonic acids or mahogany acids  
are obtained from the acid treated extract after  
each portion of sulfuric acid has been added  
thereto.

The mechanism by which the alkaline salts of petroleum sulfonic acids are effective in preventing the corrosion of copper alloys by ammonia is not understood, but it is believed to be due to the formation of a very thin protective film on the metal. It is understood, of course, that I do not wish to bind myself to any theory offered as an explanation of the beneficial effect.

An advantage of the process of the present invention, irrespective of the prevention of corrosion of copper and its alloys, is the ability to use existing equipment in which copper and its alloys are present in processes involving the use of ammonia.

In order to illustrate the beneficial effects of this invention, specimens of copper-containing metal (70% copper, 29% zinc, and 1% tin) were immersed in aqueous solutions of ammonia. These tests were in progress for 24 hours at room temperature and atmospheric pressure. Air was bubbled through the ammonia solutions throughout the tests. These tests were repeated under identical conditions with small amounts of sodium sulfonates of petroleum sulfonic acids of the type illustrated added to the aqueous solutions of ammonia. The results obtained in these tests are shown in the following table:

| Ammonium Hydroxide Solution | Material Added                        | Wt. Per Cent Based on Ammonia Sol'n | Corrosion Rate, Inch per year | Per Cent Reduction |
|-----------------------------|---------------------------------------|-------------------------------------|-------------------------------|--------------------|
| 5% by wt.                   | None                                  |                                     | 0.1425                        |                    |
| Do.                         | Sodium Sulfonates                     | 1.0                                 | 0.0682                        | 52.1               |
| Do.                         | Sulfonates of Petroleum Hydrocarbons. | 0.5                                 | 0.0268                        | 81.2               |
| Do.                         |                                       | 0.25                                | 0.0753                        | 47.2               |

It will be observed from the data presented in the foregoing table that the addition of small amounts of sodium salts of petroleum sulfonic acids effects marked reductions in the tendencies of aqueous solutions of ammonia to corrode copper-containing alloys.

Another series of runs identical to those described in the foregoing paragraph was conducted in which specimens of the same type of copper-containing metal were immersed in aqueous solutions of ammonia to which were added small amounts of ammonium sulfonates of mahogany acids from petroleum. All conditions in this series of runs otherwise were identical to the series of runs in which sodium sulfonates of mahogany acids were employed. The results obtained in these runs are shown in the following table:

| Ammonium Hydroxide Solution | Material Added                        | Wt. Per Cent Based on Ammonium Sol'n | Corrosion Rate, Inch per year | Per Cent Reduction |
|-----------------------------|---------------------------------------|--------------------------------------|-------------------------------|--------------------|
| 5% by wt.                   | None                                  |                                      | 0.1425                        |                    |
| Do.                         | Ammonium Sulfonates                   | 0.5                                  | 0.01720                       | 88.0               |
| Do.                         | Sulfonates of Petroleum Hydrocarbons. | 0.25                                 | 0.0346                        | 75.7               |
| Do.                         |                                       | 0.05                                 | 0.0418                        | 70.6               |

It will be observed from the data presented in the foregoing table that the addition of small amounts of ammonium salts of petroleum sulfonic acids effects marked reductions in the tendencies of aqueous solutions of ammonia to corrode copper-bearing alloys.

The present invention has been described and illustrated as inhibiting the corrosive effect of solutions in ammonia and water. It is understood that the invention has broad application in the inhibition of corrosive action of an ammoniacal solution such as ammonia and water to copper-bearing metals. The invention may be applied to the inhibition of the corrosive effects of aqueous solutions of ammonium salts. For example, ammonium acetate is widely used in the petroleum refinery as a solvent. It is known that ammonium acetate will attack copper-bearing metals quite readily. Therefore, it is within the spirit and scope of the invention to inhibit the corrosiveness of ammonium salt solutions to copper-bearing metals employing salts of mahogany acids as the inhibitor.

The nature and objects of the present invention having been fully described and illustrated, what I wish to claim as new and useful and to secure by Letters Patent is:

1. A method for reducing the corrosive action of a corrosive solution including ammonia, water, and oxygen to an article having a corrodible surface consisting of copper, tin, and zinc in contact with said solution which comprises introducing into said solution an amount of a salt of a petroleum mahogany acid sufficient to inhibit the corrosion thereof.
2. A method in accordance with claim 1 in which the amount of salt of mahogany acids is in the range between 0.001% and 5% by weight of the corrosive solution.
3. A method in accordance with claim 1 in which the salt of mahogany acid is a sodium salt.
4. A method in accordance with claim 1 in which the salt of mahogany acid is a potassium salt.
5. A method in accordance with claim 1 in which the salt of mahogany acid is an ammonium salt.

CECIL PHILLIPS, JR.

#### REFERENCES CITED

The following references are of record in the file of this patent:

#### UNITED STATES PATENTS

| Number    | Name          | Date          |
|-----------|---------------|---------------|
| 1,630,101 | Wilkin        | May 24, 1927  |
| 2,081,168 | De Mering     | May 25, 1937  |
| 2,238,651 | Keenen        | Apr. 15, 1941 |
| 2,349,785 | Faust         | May 23, 1944  |
| 2,445,936 | Butcosk       | July 27, 1948 |
| 2,455,659 | Duncan et al. | Dec. 7, 1948  |